

## UNITED STATES PATENT OFFICE

2,286,626

## ALUMINUM BASE ALLOY

Louis W. Kempf and Walter A. Dean, Lakewood, Ohio, assignors to Aluminum Company of America, Pittsburgh, Pa., a corporation of Pennsylvania

No Drawing. Application December 30, 1941,  
Serial No. 424,893

2 Claims. (Cl. 75—146)

This invention relates to aluminum base alloys that are especially adapted for use at elevated temperatures.

Most of the applications where aluminum base alloys are employed involve exposure to the usual atmospheric temperature range. However, there are places where it is necessary to use aluminum alloy parts at elevated temperatures, for example, in internal combustion engines. Some of the parts are exposed to temperatures within the range of 400 to 600° F. The demand for light alloys which can be employed at elevated temperatures has been increased by the demand for more powerful motors for aircraft. It is an object of this invention to provide an alloy composition which exhibits high strength and resistance to deformation at elevated temperatures, especially at the higher temperatures found in the newer aircraft motors. A particular object is to provide an alloy which possesses a high thermal conductivity along with the high strength at elevated temperatures. Still another object is to provide an aluminum base alloy having a higher modulus of elasticity than the common aluminum base alloys now in use.

We have discovered that an aluminum base alloy containing from about 20 to 40 per cent beryllium, from 0.25 to 3 per cent magnesium, from 2 to 15 per cent zinc, and the balance substantially aluminum possesses the aforementioned properties. More particularly, we have found that some of the alloys within this range possess tensile strengths at elevated temperatures which are considerably greater than that of alloys heretofore used for such service. The presence of zinc in the alloys increases their susceptibility to improvement in strength, solution heat treatment and age hardening as compared to the same alloys without zinc. Furthermore, this increase in strength is accompanied by a lower density than aluminum, a relatively high thermal conductivity, and a high modulus of elasticity. This combination of properties, especially that of high strength, and relatively high thermal conductivity, makes the alloys particularly useful for such articles as valve push rods, pistons, and the like which are highly stressed at elevated temperatures. The high modulus of elasticity of these alloys makes it possible to design structures having a greater resistance to distortion under a load with a given section thickness or the same resistance to distortion with a lighter section as compared to structures made from alloys having lower modulus values. Our alloys may be used in either cast or wrought form but we prefer to use them in wrought form.

5 The tensile properties at an elevated temperature of some examples of our alloys, and the thermal conductivity at room temperature of two of these alloys, together with the corresponding properties of certain well known aluminum base alloys which have been used heretofore for high temperature service, are given in Table I below. The first of the two alloys which contained no beryllium, i. e. the Al-Cu-Ni-Mg alloy, may be considered as being typical of aluminum base alloys designed for service at elevated temperatures. The balance of the composition of each of the alloys appearing in the tables was aluminum and the usual impurities. The beryllium-containing alloys were cast as ingots and extruded into the form of rods.

10 The thermal conductivity and tensile property determinations were made on specimens taken from extruded rods while the test specimens of the other aluminum base alloys were taken from forged rods. The difference in fabricating practices used in making the rods is considered to have no significant effect upon the test results reported here. The specimens without beryllium received the conventional solution heat treatment and artificial aging before being subjected to any of the treatments and tests herein described in order to duplicate the condition of the alloys in many commercial applications. Specimens of the last beryllium-containing alloy in 15 Table I likewise received a solution heat treatment and artificial aging. All of the test bars for tensile strength determinations were subjected to a short time test at elevated temperatures consisting of first stabilizing them by heating them for 16 hours at 700° F. This preliminary treatment served to accelerate any changes which would have occurred on exposure to a lower temperature over a long period of time. We have found from a number of other tests that such preliminary stabilizing treatment for 20 a relatively short period of time at a temperature higher than encountered in service affects properties to a comparable extent as more extended periods at the temperature of service operation. Following the preliminary stabilizing treatment, the bars for tensile strength determinations were cooled to room temperature, then reheated to the testing temperature, in this case 600° F., held 25 at this temperature for one-half hour, and then broken in tension at 600° F. in the usual manner.

30 The thermal conductivity values were calculated from electrical resistivity measurements made at room temperature. The calculations were based on the well recognized Wiedemann-

Franz-Lorenz relationship between the thermal conductivity and electrical resistivity of metals. It is generally true that there is such a small change in thermal conductivity of aluminum base alloys over the range of room temperature to about 600° F. that values at room temperature are very close to those at elevated temperatures such as exist in internal combustion engines. The test specimens for electrical resistivity measurements were in the same temper as that of the specimens used for tensile tests prior to the stabilizing treatment.

from these data. From other determinations we have had made at elevated temperatures, we have found that the alloys containing beryllium retain this superiority by a wide margin. The relatively high modulus at elevated temperatures means that structures made from such alloys are much more resistant to distortion and hence may be expected to give longer service.

It has been our experience that a substantial amount of beryllium must be present to obtain the combination of properties described above. A minimum of about 20 per cent of this element

TABLE I  
Tensile properties at 600° F. and thermal conductivity at room temperature

| Alloy composition |         |         |         |         | Tensile strength | Elongation in 2 inches | Thermal conductivity (C. G. S. units) |
|-------------------|---------|---------|---------|---------|------------------|------------------------|---------------------------------------|
| Be                | Mg      | Zn      | Ni      | Si      | Lbs./sq. in.     | Percent                | Percent                               |
| Percent           | Percent | Percent | Percent | Percent |                  |                        |                                       |
| 24.15             | 0.56    | 5.21    |         |         | 8,600            | 17                     | 0.38                                  |
| 24.09             | 0.63    | 9.97    |         |         | 8,200            | 14                     |                                       |
| 39.41             | 0.35    | 11.40   |         |         | 10,000           | 8                      | 0.32                                  |
| 28.65             | 0.87    | 3.43    |         |         | 13,900           | 8.5                    |                                       |
|                   | 0.5     | 4.0     | 2.0     |         | 6,000            | 75                     | 0.37                                  |
|                   | 1.0     | 0.9     | 0.9     | 12.5    | 5,600            | 54                     | 0.32                                  |

It will be noted that the tensile strength of the beryllium-containing alloys at the elevated temperature exceeds that of the two aluminum base compositions used for comparison. The lower elongation values of the beryllium alloys also indicate a greater resistance to deformation at elevated temperatures. These tensile properties therefore indicate that these alloys are much better adapted for service at such high temperatures as 600° F. than the other two aluminum base alloys which have been employed heretofore for that purpose. It is also to be observed that the thermal conductivities of the alloys containing 24.15 and 29.41 per cent beryllium are substantially the same as those of the two alloys containing no beryllium. A thermal conductivity of 0.3 c. g. s. units, or more, is considered to be relatively high for alloys used at elevated temperatures.

Modulus of elasticity determinations were made at room temperature on two alloys containing 24.09 and 22.10 per cent beryllium, respectively, and on three common aluminum base alloys containing no beryllium. The alloys containing beryllium were tested in the as-extruded condition, while the other alloys were given a solution heat treatment and artificial aging. As is well recognized, such a difference in condition of the alloys would not affect the modulus values. The test results are given below in Table II:

TABLE II  
Modulus of elasticity at room temperature

| Alloy composition |         |         |         |         |         |         | Modulus      |
|-------------------|---------|---------|---------|---------|---------|---------|--------------|
| Be                | Mg      | Zn      | Cu      | Mn      | Ni      | Si      | Lbs./sq. in. |
| Percent           | Percent | Percent | Percent | Percent | Percent | Percent |              |
| 22.10             | 0.70    | 5.14    |         |         |         |         | 16,700,000   |
| 24.09             | 0.63    | 9.97    |         |         |         |         | 17,400,000   |
|                   | 0.4     | 10.0    | 1.0     | 0.75    |         |         | 10,300,000   |
|                   | 0.5     |         | 4.0     |         | 2.0     |         | 10,300,000   |
|                   | 1.0     |         | 0.9     |         | 0.9     | 12.5    | 10,300,000   |

The superiority of the beryllium-containing alloy over the other alloys is readily apparent

30 has been found to be necessary to obtain such a combination of properties, but that if more than 40 per cent is employed, the alloy becomes very difficult to work. The presence of magnesium in the alloy considerably enhances the strength 35 and resistance to fatigue at elevated temperatures. We have found that at least 0.25 per cent magnesium is necessary to achieve this purpose, while on the other hand, if more than 3 per cent is used, fabricating difficulties are encountered. 40 The addition of zinc serves to increase the susceptibility of the alloys to improvement in strength by solution heat treatment and age hardening as compared to the same alloys without zinc, and the greatest benefit in this respect 45 is obtained by using from 2 to 15 per cent of this element. Alloys which contain from 22 to 30 per cent beryllium, 0.5 to 1.5 per cent magnesium, and 2.5 to 10 per cent zinc are preferred because they possess the most satisfactory combination of strength and workability.

50 The expression "balance substantially aluminum", as used hereinabove and in the appended claims, means that small amounts of the usual impurities as well as other elements may be present in the alloys without affecting the high temperature properties described above. The presence of any elements which substantially impair the strength and thermal conductivity properties of these alloys at elevated temperatures are therefore excluded from the scope of this invention.

55 In referring to certain properties of our alloys at elevated temperatures we mean that these properties are particularly outstanding in the range of 400 to 600° F., however, the advantageous properties of our alloys are not confined to that temperature range.

60 The examples of the beryllium-containing alloys given hereinabove are for the purpose of illustrating our invention and are not to be regarded as limiting its scope. Other alloy compositions within the range set forth above possess equally satisfactory properties at elevated temperatures.

We claim:

1. An aluminum base alloy consisting of from about 20 to 40 per cent beryllium, 0.25 to 3 per cent magnesium, 2 to 15 per cent zinc, and the balance substantially aluminum, said alloy being characterized by a high tensile strength at elevated temperatures combined with a relatively high thermal conductivity, and a greater susceptibility to improvement in strength by solution heat treatment and age hardening than the same alloy devoid of zinc.

2. An aluminum base alloy adapted for service

5 at elevated temperatures consisting of from 22 to 30 per cent beryllium, 0.5 to 1.5 per cent magnesium, 2.5 to 10 per cent zinc, and the balance substantially aluminum, said alloy being characterized by a high tensile strength at elevated temperatures combined with a relatively high thermal conductivity, and a greater susceptibility to improvement in strength by solution heat treatment and age hardening than the same alloy devoid of zinc.

LOUIS W. KEMPF.  
WALTER A. DEAN.

CERTIFICATE OF CORRECTION.

Patent No. 2,286,626.

June 16, 1942.

LOUIS W. KEMPF, ET AL.

It is hereby certified that error appears in the printed specification of the above numbered patent requiring correction as follows: Page 2, Table I, first column thereof, for "39.41" read --29.41--; and same page, first column, line 32, for "aluminium" read --aluminum--; and that the said Letters Patent should be read with this correction therein that the same may conform to the record of the case in the Patent Office.

Signed and sealed this 4th day of August, A. D. 1942.

Henry Van Arsdale,  
(Seal) Acting Commissioner of Patents.